

# UNITED STATES PATENT OFFICE.

ALBERT E. STRIPPEL, OF NEW YORK, N. Y.

## STENCIL FABRIC AND PROCESS OF PRODUCING THE SAME.

1,169,520.

Specification of Letters Patent.

Patented Jan. 25, 1916.

No Drawing. Original application filed July 1, 1913, Serial No. 776,893. Divided and this application filed February 17, 1914. Serial No. 819,296.

*To all whom it may concern:*

Be it known that I, ALBERT E. STRIPPEL, a citizen of the United States, and resident of the borough of Manhattan, in the city 5 and State of New York, have invented a new and useful Improvement in Stencil Fabrics and Processes of Producing the Same, of which the following is a specification.

The objects of my invention are to produce a stencil fabric which will be very durable and sufficiently strong to withstand the severe treatment to which it is subjected in use; which will prevent the type for cutting the stencils from cutting completely 15 through the fabric and blocking out closed characters and which will provide a clear print.

The fabric which is most suitable to be treated to render it desirable as a stencil 20 fabric is a long fiber fabric such as is commonly used in this art, as, for instance, Japanese dental paper. This fabric may be used either in a single thickness or a multiple thickness as desired and it is pasted 25 along one edge in the usual manner upon a suitable holder of waterproof material for convenience in handling the fabric during its treatment. After the fabric has been completed ready for use, it may be cut into 30 the required sizes for use and cemented on the usual cardboard or fiber frames.

The stencil fabric consists of a long fiber fabric provided with a hygroscopic film rendered impervious to the action of the oils 35 contained in printing inks. While this would produce a stencil fabric which could be used for a short time still to produce a durable stencil, it is necessary to keep this film in a soft and pliable state and also to 40 protect it from deterioration for otherwise it would become brittle and crack when handled or run through an addressing machine and it would also be subject to decay. This stencil fabric has heretofore been treated 45 with an organic oil and a preservative, as, for instance, glycerin and formaldehyde.

The object of this invention is to produce a stencil fabric which will be superior to those heretofore produced as to pliability, 50 durability, and strength. This result is accomplished by the use of metallic salts which are perfectly soluble in water and inorganic acids but not in organic oils, so that they will not be affected by the ink solu-

tions. This method of preservation by the use of metallic salts has proved to be much superior to the former preservation method above referred to.

Where a solution containing gelatin and bichromate of potash is subjected to the presence of light, it has a tendency to thicken, due to the chemical action between the gelatin and the chrome salt whereby the gelatin is rendered insoluble. Heretofore, to keep this solution in a good working degree 60 of fluidity, it has been necessary to exclude it from the action of light which makes the process very difficult and expensive. I have discovered that by the use of a hygroscopic nitrate, such as sodium nitrate, I can expose 65 the solution to the light and yet keep the specific gravity of the solution practically constant, for the reason that the nitrate has the effect of materially retarding the setting of the film. The nitrate is not affected 70 by the setting of the film and in the finished product it aids in keeping the paper moist by drawing moisture from the atmosphere along with the chlorid. It also preserves 75 the paper from deterioration by the action of 80 microbes which is the only natural process by which the gelatin and glycerin can be destroyed.

In producing a stencil fabric which will not require moistening before being used, 85 the process is carried out as follows:—I dissolve 16 ounces of a colloid of animal origin, such as gelatin, in 5 pints of water and heat the same up to approximately 140° F., and maintain the solution at this temperature, 90 as, for instance, in a water bath. Should the gelatin have a tendency to leave an insoluble residue, it is desirable to strain the solution. After the gelatin has been thoroughly dissolved, I add thereto from 18 to 95 22 ounces of glycerin and 1.5 ounces of a hygroscopic nitrate, such as sodium nitrate, and mix the parts thoroughly. In a separate vessel I dissolve from .48 of an ounce to .32 of an ounce of a chrome salt, such as 100 bichromate of potash, in 5 pints of water so that the weight of the chrome salt will be between 3½% and 3% of the weight of the gelatin. The smaller the percentage of chrome salt, the softer will be the setting 105 of the film. This solution is heated to 140° F., and added to the solution of gelatin, glycerin and sodium nitrate. The sheet of

long fiber fabric is run through the solution of gelatin, glycerin, sodium nitrate and bichromate of potash, and then the excess of the solution is squeezed from the sheet, as, 5 for instance, by passing the sheet through cold pressure rollers. The sheet is then hung up a sufficient time to only partially dry and is then again run through the solution of gelatin, glycerin, sodium nitrate and 10 bichromate of potash, and the excess solution removed therefrom. The minimum amount of bichromate of potash and the maximum amount of glycerin should be used to produce the best results. The 15 sheet is then hung up for about twenty-four hours and is then placed upon a suitable non-porous surface, such as glass, and a solution of glycerin is applied thereto by any suitable means, such as a brush or roller. 20 To this solution, I may add alcohol and aluminum chlorid. The solution which I have found very suitable is one comprising substantially the following proportions, by weight: water, 16 parts; glycerin, 5 parts; 25 alcohol, 1 part; and aluminum chlorid, 1 part. The sheet is then again hung up to dry and may thereafter be cut into the required sizes for use. A stencil fabric produced by this method, will produce a clear 30 print which is not the case with the stencils of this type heretofore produced, said stencils requiring a number of impressions before beginning to produce a legible print. The film is also kept in such a condition that 35 the type will not cut completely through the fabric and block out inclosed characters.

This application is a division of United States Letters Patent No. 1,092,509, dated April 7, 1914, the application for which was 40 filed July 1, 1913, Serial No. 776,893.

What I claim is:

1. The process of producing a stencil fabric which consists in treating a long fiber fabric, first, with a solution of a colloid of 45 animal origin, glycerin, a hydroscopic nitrate and a chrome salt; second, partially drying the fabric; third, again treating the fabric with the said solution; fourth, drying the fabric; fifth, applying thereto a solution 50 of glycerin; and sixth, again drying the fabric.

2. The process of producing a stencil fabric which consists in treating a long fiber fabric, first, with a solution of a colloid of 55 animal origin, glycerin, a hydroscopic nitrate and a chrome salt; second, partially drying the fabric; third, again treating the fabric with the said solution; fourth, drying the fabric; fifth, applying thereto a solution 60 of glycerin, alcohol and aluminum chlorid; and sixth, again drying the fabric.

3. The process of producing a stencil fabric which consists in treating a long fiber fabric, first, with a solution of a colloid of 65 animal origin, glycerin, a hydroscopic ni-

trate and a chrome salt; second, partially drying the fabric; third, again treating the fabric with said solution; fourth, drying the fabric; fifth, applying thereto a solution of glycerin, alcohol and aluminum chlorid 70 in substantially the following proportions, by weight; glycerin, 5 parts; alcohol, 1 part; aluminum chlorid, 1 part; and sixth, again drying the fabric.

4. The process of producing a stencil fabric which consists in treating a long fiber fabric, first, with a solution of gelatin, glycerin, sodium nitrate and bichromate of potash; second, partially drying the fabric; 75 third, again treating the fabric with the said solution; fourth, drying the fabric; fifth, applying thereto a solution of glycerin; and sixth, again drying the fabric.

5. The process of producing a stencil fabric which consists in treating a long fiber 80 fabric, first, with a solution of gelatin, glycerin, sodium nitrate and bichromate of potash; second, partially drying the fabric; third, again treating the fabric with the said solution; fourth, drying the fabric; fifth, 85 applying thereto a solution of glycerin, alcohol and aluminum chlorid; and sixth, again drying the fabric.

6. The process of producing a stencil fabric which consists in treating a long fiber 90 fabric, first, with a solution of gelatin, glycerin, sodium nitrate and bichromate of potash; second, partially drying the fabric; third, again treating the fabric with the said solution; fourth, drying the fabric; fifth, 95 applying thereto a solution of glycerin, alcohol and aluminum chlorid in substantially the following proportions, by weight; glycerin, 5 parts; alcohol, 1 part; aluminum chlorid, 1 part; and sixth, again drying the 100 fabric.

7. The process of producing a stencil fabric which consists in treating a long fiber fabric, first, with a solution of gelatin, glycerin, sodium nitrate and bichromate of potash, in substantially the following proportions by weight: gelatin, 16 ounces; glycerin, 18 to 22 ounces; sodium nitrate 1.5 ounces and bichromate of potash .48 to .32 of an ounce; second, partially drying the 110 fabric; third, again treating the fabric with the said solution; fourth, drying the fabric; fifth, applying thereto a solution of glycerin; and sixth, again drying the fabric.

8. The process of producing a stencil fabric which consists in treating a long fiber fabric, first, with a solution of gelatin, glycerin, sodium nitrate and bichromate of potash in substantially the following proportions, by weight: gelatin, 16 ounces; glycerin, 18 to 22 ounces; sodium nitrate, 1.5 ounces and bichromate of potash .48 to .32 of an ounce; second, partially drying the fabric; third, again treating the fabric with the said solution; fourth, drying the fabric; 125

fifth, applying thereto a solution of glycerin, alcohol and aluminum chlorid; and sixth, again drying the fabric.

9. The process of producing a stencil fabric which consists in treating a long fiber fabric, first, with a solution of gelatin, glycerin, sodium nitrate and bichromate of potash in substantially the following proportions, by weight: gelatin, 16 ounces; glycerin, 18 to 22 ounces; sodium nitrate, 1.5 ounces and bichromate of potash .48 to .32 of an ounce; second partially drying the fabric; third, again treating the fabric with the said solution; fourth, drying the fabric;

fifth, applying thereto a solution of glycerin, alcohol and aluminum chlorid in substantially the following proportions, by weight: glycerin, 5 parts; alcohol, 1 part; aluminum chlorid, 1 part; and sixth, again drying the fabric.

In testimony, that I claim the foregoing as my invention, I have signed my name in presence of two witnesses, this twenty-seventh day of January, 1914.

ALBERT E. STRIPPEL.

Witnesses:

F. GEORGE BARRY,  
C. S. SUNDGREN.